

Oct. 29, 1935.

E. AYRES ET AL

2,019,037

MANUFACTURE OF IMPROVED HYDROCARBON PRODUCTS

Filed March 10, 1932

Fig. 1.



Inventors

Eugene Ayres,  
Herschel G. Smith,

By K.P. McElroy  
Attorney

## UNITED STATES PATENT OFFICE

2,019,037

## MANUFACTURE OF IMPROVED HYDRO-CARBON PRODUCTS

Eugene Ayres and Herschel G. Smith, Swarthmore, Pa., assignors to Gulf Refining Company, Pittsburgh, Pa., a corporation of Texas

Application March 10, 1932, Serial No. 598,096

6 Claims. (Cl. 196—78)

This invention relates to manufacture of lubricating oils; and it comprises a process of producing finished high quality lubricating oils from mixtures of technical petroleum stocks ranging 5 in type from tar residues to light distillates, wherein a relatively high boiling petroleum stock is mixed with a lower boiling stock, the mixture is heated to a temperature not above 300° F. in the presence of anhydrous aluminum chlorid 10 and added HCl to produce a synthetic stock of characteristics intermediate those of the two original stocks and in yield much greater than is obtainable by a similar treatment applied to the original stocks separately, the synthetic stock 15 which contains some aluminum chlorid sludge is settled for removal of the bulk of sludge, is decanted, traces of aluminum chlorid sludge remaining in suspension in the decanted liquid are decomposed and the products of decomposition 20 are substantially completely removed, to produce a finished lubricating oil substantially free from impurities; all as more fully hereinafter set forth and as claimed.

Several different, specific effects of anhydrous 25 aluminum chloride on petroleum stocks have been described in the literature. A few of these effects now form the basis of commercial processes. For example, it is known that aluminum chlorid has the effect of causing the condensation or polymerization of hydrocarbons at relatively moderate 30 temperatures. By this means, synthetic lubricating oils of naphthenic type have been made from volatile olefines. The refining of lubricating oil stocks by warming with aluminum chloride is also known. Such processing involves the 35 removal in the form of a heavy sludge of certain undesirable constituents of the stock, possibly by the condensation of the constituents least saturated with respect to hydrogen to form high molecular weight compounds insoluble in oil. It is characteristic of such processes that the oil is changed in character; they break down the 40 molecular structure of the oil and produce the formation of substantial proportions of oils of lower viscosity than that of the starting material. The reason for this breaking down effect is that the aluminum chloride of itself is not ordinarily an effective refining agent unless the temperature 45 of the oil is above normal. In any event a considerable amount of the starting stock is lost to the sludge and the yield of refined oil is low.

A third example of the known effects of aluminum chlorid is the use of this material to promote the breaking down of heavier oils to form 50 motor fuel and kerosene. At temperatures above 300° F. the analytic or converting effect of aluminum chlorid predominates, and at temperatures below 300° F. the synthetic effect of aluminum chlorid, although dominating the analytic ef-

fect, may cause the formation of oil insoluble bodies in large amounts.

In the present invention in its aspect of producing a synthetic lubricating oil stock in high yield, aluminum chlorid in the presence of added 5 HCl is used for synthesizing lubricating oils from mixtures of hydrocarbon stocks. In the principal embodiment of the invention, a relatively thick, viscous and high boiling oil stock is admixed with a lighter stock. In the course of treatment, some 10 sort of combination of the stocks takes place. There is, to a certain extent, what may be called an averaging of the two oils; and the new oil produced therefrom may be termed a synthetic product. That this synthesizing effect occurs 15 is evidenced by the fact that the yield of oil obtained in the process is much greater than the sum of the yields obtained by carrying out a similar process upon the two components separately and mixing the products. 20

The HCl as used in our process appears to have a transitory function. The entire chlorine content of the gas appears at the end of the reaction as hydrogen chloride. No chlorinated hydrocarbons appear in the product. The hydrogen chloride can be readily recovered at the 25 end of the reaction and can then be reintroduced or recycled.

Our synthesizing process is carried out upon mixtures of hydrocarbons of different characteristics. In the principal embodiment of the invention, the two hydrocarbon components are a high boiling petroleum stock and a lower boiling stock. To the extent that the two stocks combine 30 molecularly, the yield of high grade products is higher than the yield obtainable from a treatment of the charging stocks separately. When one of the hydrocarbon components is of low molecular weight, its presence has an additional 35 effect: a thinning action; ensuring, by dilution of 40 viscous oils, better contact with the aluminum chlorid.

In general, our process is accomplished by contacting dry hydrogen chloride, for example, with the hydrocarbon stock to be treated, adding a 45 suitable proportion of anhydrous aluminum chloride, agitating at a suitable temperature for a suitable period of time, separating the sludge from the residual oil, neutralizing the separated oil and finishing in such manner as to obtain the 50 desired appearance or purity of product.

The contacting of the oil with dry gaseous hydrogen chloride in our process can be accomplished conveniently at ordinary temperatures and pressures, but elevated pressures may be 55 advantageous particularly when elevated temperatures are employed. Pressures up to 100 pounds per square inch have been used in some cases. The oil may be merely held in contact with an atmosphere of the hydrogen chloride, 60

with or without agitation, or the latter may be blown through a body of the oil. When atmospheric pressure is used it is advantageous to maintain the contact with hydrogen chloride for 5 an hour or more. At slightly elevated temperatures and under super-atmospheric pressures the same degree of preparation of the hydrocarbon stock may be accomplished within 5 to 10 minutes. It is advantageous, although not necessary 10 to maintain contact with excess hydrogen chloride during the subsequent treatment with aluminum chloride. Aluminum chloride in its reaction with hydrocarbons generates some hydrogen chloride but we have found that the small amount 15 of hydrogen chloride so generated is not capable of giving the results obtainable by this invention. An excess over this amount is necessary. It has also been found that the aluminum chloride used in our process cannot be replaced by metallic 20 aluminum used with  $\text{Cl}_2$  or  $\text{HCl}$ . If there is a reaction between such aluminum and the dry hydrogen chloride or chlorine used in our process, this reaction is, at all events, not sufficiently rapid. The results are not the same. 25 Instead of contacting the hydrocarbon stock with hydrogen chloride prior to treatment with aluminum chloride, satisfactory results may be secured by contacting with hydrogen chloride only during the treatment with aluminum chloride, provided this treatment is conducted at 30 moderate temperatures.

We have found it practical in some instances to substitute gaseous chlorin for the  $\text{HCl}$  gas used in our process prior to or during treatment of stock 35 with aluminum chloride. So doing, the net result appears to be the same; the chlorine is quantitatively removed at the end of the reaction as  $\text{HCl}$ . Operation is under conditions such that no substantial chlorination of the hydrocarbons present 40 takes place.

The proportion of anhydrous aluminum chloride used in our process may be varied within wide limits. We advantageously use between 1 and 10 per cent by weight of the hydrocarbon 45 stock. In the processes illustrated subsequently 1 per cent of aluminum chloride was found sufficient to give a 94 per cent yield of a slightly improved lubricating oil with a viscosity at 210° F. of 86 seconds compared with 75 for the starting material, which in this case was a lubricating stock from a Coastal crude. But with the use of 50 10 per cent aluminum chloride and the same lubricating stock, the viscosity at 210° F. of the finished product was raised to 107 seconds and the quality approached that of Pennsylvania oil, with an 87 per cent yield. Larger proportions of 55 aluminum chloride are usually attended by larger losses. The effects on the reduction of carbon residue are more marked at higher temperatures 60 with larger proportions of aluminum chloride, but at lower temperatures relatively little aluminum chloride is required. With 3 per cent aluminum chloride at room temperature the carbon residue of a mid-continent bright stock with a viscosity 65 at 210° F. of 150 seconds can be reduced from 1.75 to 0.55, for example.

By the use of an excess of hydrogen chloride much less aluminum chloride is required than in the ordinary known process. The temperatures 70 suitable for our processes vary between those considerably below room temperature and those somewhat above 212° F. Temperatures above 300° F. are not satisfactory because at elevated temperatures the action of aluminum chloride 75 is to break down the hydrocarbons to form light

hydrocarbons instead of building up or maintaining the viscosities according to the present invention. In the case of relatively low hydrogen : carbon ratio hydrocarbon stocks, the maximum effect on the viscosity-temperature relationship appears to be at low temperatures, whereas with relatively high hydrogen : carbon ratio hydrocarbon stocks, higher temperatures produce better results.

The time of agitation of the hydrocarbon stock 10 with aluminum chloride should be long enough to insure a complete reaction. At low temperatures it is obviously advantageous to use a longer time than at high temperatures. In general a period of one hour gives satisfactory results.

The dilution of the hydrocarbon stock with low molecular weight hydrocarbons is advantageous in the case of the treatment of hydrocarbons of higher molecular weight and particularly of viscous oils. For example, in the treatment 20 of pressure-still tar alone there is obtained a 33 per cent yield of good quality oil with a viscosity of 42 seconds at 210° F., whereas in the presence of an equal part of a cracked gasoline a 25 97 per cent yield may be obtained of oil of the same quality and viscosity. On the other hand after a treatment of the cracked gasoline separately, conditions of treatment being otherwise the same, no measurable yield of lubricating oil was secured. The treatment of a mid-continent 30 bright stock alone gives a 60 per cent yield of oil of Pennsylvania quality with viscosity of 85 seconds at 210° F., but in the presence of 20 per cent uncracked mid-continent gasoline we obtain a 65 per cent yield of oil of Pennsylvania 35 quality with viscosity of 143 seconds (S. U. V.).

The chemical characteristics of the diluent have a marked effect on the results, but all types are useful. Pure olefines such as amylenes may be used to advantage. Cracked gasolines containing 40 ring compounds as well as olefines and uncracked gasolines containing principally paraffins and naphthenes, or even pure benzene or toluene, or any combinations of these hydrocarbons, may be used. The increase in yield is somewhat more 45 marked with diluents of the olefine type. This is not because of a polymerization or condensation of the olefins to form an oil, by the action of aluminum chloride, because a treatment of the olefine alone under the prescribed conditions gives 50 no measurable yield of lubricating oil.

In the case of the treatment of certain types of stocks by our process, particularly those types that contain unsaturated lubricating fractions or naphthene lubricating fractions, we often secure lubricating oils that are mixtures of oils of improved quality with some fractions of inferior quality. The formation of refined lubricating oil fractions of poorer quality appears to be the result of side reactions, with polymerization or condensation of heavy hydrocarbons to products having the undesirable characteristics of low gravities, poor viscosity-temperature curves, and comparatively high carbon residue tests. These side reactions or by-products occasionally 65 encountered are evidently largely due to the presence of substances in the charging stocks of the nature of hydrocarbons of the di-olefine, acetylenic or aromatic types. When such reaction products are encountered in sufficient 70 amount to affect the quality of the finished lubricating oil mixture to an undesirable extent, we can often effect some improvement in quality by distilling from the final treated oil, fractions of improved quality, as the undesirable products are 75

often of much higher boiling range than the other fractions and therefore can be concentrated in a heavy residual oil from a fire and steam reduction at either atmospheric pressure or under 5 vacuum.

The intermediate stock obtained by the treatment described of a mixture of charging stocks with the aid of aluminum chloride and added HCl, is not a finished lubricating oil and cannot be 10 used directly as such. It is necessary to apply a finishing treatment to get out all traces of aluminum chloride, or aluminum chloride sludge, remaining in the synthesized stock. The stocks do not yield readily to treatment by common methods 15 for finishing oils in general and we have developed methods particularly suitable for finishing such stocks. Three finishing methods which we have found most suitable, for producing a finished oil from synthetic stocks are the following:—

20 1. To the sour oil decanted from the aluminum chloride sludge is added some fine clay and hydrated lime, the oil thereafter being filtered. Heating of the oil-lime-clay mixture before filtering is usually advantageous. Two-tenths of a 25 pound of lime per barrel of oil per acid number is about sufficient for neutralization, but it is desirable to use an excess such as 0.6 pound per barrel per acid number. Sufficient clay should be used to facilitate filtration. This usually requires 30 from 0.4 to 0.8 pound of clay per gallon of oil, when natural Florida or Georgia clay is employed.

2. The sour oil decanted from the aluminum chloride sludge is agitated with dilute sulfuric acid to decompose suspended aluminum chloride 35 sludge or compounds. After settling out the dilute acid wash, the oil may be treated, if desired, with a small amount of strong sulfuric acid, or contacted with fine clay, or filtered through coarse burned clay. The dilute acid may be as weak as 5 40 per cent or less, or may be stronger than 20 per cent unless, in a particular case, the strong acid causes a stable suspension in the oil of acid sludge particles or decomposition products therefrom.

45 3. The sour oil decanted from the aluminum chloride sludge is heated to a temperature at which the traces of suspended aluminum chloride sludge will completely react with the oil. This temperature is usually between 450° F. and 550° F. After the sludge is spent, the oil can be satisfactorily filtered.

50 Our invention is illustrated in the accompanying drawing which shows, in the form of flow sheets (Figs. 1 and 2), two typical processes within the purview of our invention, wherein a lubricating oil stock is mixed with a lighter hydrocarbon and the mixture is treated by a series of successive operations with the ultimate production 55 of a finished lubricating oil of improved properties. The several successive operations are indicated on the flow sheets by appropriate legends.

60 Referring to the flow sheet of Fig. 1, a lubricating oil stock is shown introduced into an agitator together with a light fraction. Aluminum chloride is introduced and hydrogen chloride is circulated through the agitator. Sludge is drawn off after completion of the reaction and the remaining sour oil is introduced into a still together with clay and sufficient lime to neutralize the 65 acidity in the oil. A light distillate is obtained from the still while the bottoms are passed through a filter press for removal of clay and lime residues, a finished lubricating oil being finally recovered.

Fig. 2 shows a modification of the invention, the finishing steps being different. The treatment with aluminum chloride and HCl is the same as in Fig. 1. The sour oil obtained at the end of this treatment is settled and is then mixed with a 5 suitable quantity of dilute sulfuric acid with agitation. The oil is then permitted to settle out impurities, and is contacted with fine clay or filtered through coarse burned clay. A finished lubricating oil of high quality is recovered by this 10 treatment.

15 Our invention is further illustrated by the following illustrative examples which represent practical embodiments thereof.

#### 1. Treatment of mid-continent bright stock

20 One hundred volumes of a bright stock from Oklahoma crude petroleum were contacted with dry hydrogen chloride at ordinary temperature and pressure for four hours. While continuing 20 the contact of hydrogen chloride, the oil was then warmed to 275° F. and stirred for about 2 hours with 10 per cent by weight of anhydrous aluminum chloride. The sludge was permitted to settle and the decanted sour oil was steamed at 25 450° F. with 0.5 pound fine clay per gallon and 0.6 pound hydrated lime per acid number per barrel. The residue was filtered through paper. The yield of finished oil was found to be 60 volumes. The following table shows comparative tests 30 made on the charging stock and on the final products.

|                                   | Charging stock | Product | 35 |
|-----------------------------------|----------------|---------|----|
| Gravity: °A. P. I.                | 22.8           | 29.9    |    |
| Viscosity, S. U. V.:              |                |         |    |
| 100° F.                           | 3,007          | 846     |    |
| 210° F.                           | 158            | 85      |    |
| Viscosity index (Dean and Davis): | 85             | 105     |    |
| Flash, O. C.: °F.                 | 545            | 420     | 40 |
| Fire, O. C.: °F.                  | 605            | 505     |    |
| Pour: °F.                         | +15            | +25     |    |
| Color, N. P. A.                   | 4.75           | 1.75    |    |
| Carbon residue: Per cent          | 1.42           | 0.04    |    |

45 The above tests show a greater effect on the viscosity index than is normally secured.

#### 2. Treatment of mid-continent bright stock

50 One hundred volumes of a bright stock from Oklahoma crude petroleum were mixed with fifty-five volumes of amylene, and contacted for two hours at ordinary temperature and pressure with dry hydrogen chloride. The oil was then stirred at room temperature with 3 per cent by weight 55 of anhydrous aluminum chloride for 4 hours at normal pressure while maintaining an atmosphere of dry hydrogen chloride over the reaction mixture. The sludge was permitted to settle and the decanted sour oil was treated as in the first 60 example. The yield of finished oil was 149 volumes. Comparative tests on this oil yielded the following results:

|                                    | Charging stock | Product | 65 |
|------------------------------------|----------------|---------|----|
| Gravity: °A. P. I.                 | 23.0           | 24.3    |    |
| Viscosity, S. U. V.:               |                |         |    |
| 100° F.                            | 3,264          | 2,059   |    |
| 210° F.                            | 151            | 119     | 70 |
| Viscosity, index (Dean and Davis): | 73             | 78      |    |
| Flash, O. C.: °F.                  | 545            | 495     |    |
| Fire, O. C.: °F.                   | 630            | 570     |    |
| Pour: °F.                          | +15            | +15     |    |
| Color, N. P. A.                    | 7.5            | 7.5     |    |
| Carbon residue: Per cent           | 1.75           | 0.55    |    |

This example illustrates a remarkably high yield of oil of reduced carbon residue.

*3. Treatment of lubricating distillate from Coastal crude*

On hundred volumes of lubricating distillate from Coastal crude petroleum were mixed with twenty-eight volumes of amylene. This mixture was contacted, with dry hydrogen chloride at room temperature while stirring with 10 per cent by weight of anhydrous aluminum chloride for a period of 4 hours. The sludge was permitted to settle and the sour oil was then treated as outlined in the first example. The yield of finished oil was found to be 86.6 volumes having the following comparative tests:

|                                  | Charging stock | Product |
|----------------------------------|----------------|---------|
| 20 Gravity: °A. P. I.            | 20.6           | 26.4    |
| Viscosity, S. U. V.: 100° F      | 1,248          | 1,548   |
| 210                              | 75             | 107     |
| Viscosity index (Dean and Davis) | 18             | 88      |
| Flash, O. C.: °F                 | 445            | 510     |
| 25 Fire, O. C.: °F               | 495            | 580     |
| Pour, °F                         | -10            | -5      |
| Color, N. P. A.                  | 4.75           | 3.0     |
| Carbon Residue: Per cent         | 0.23           | 0.30    |

This example shows a great increase in viscosity index attended by an increase in viscosity at 210° F.

*4. Treatment of reduced pressure-still tar*

One hundred volumes of reduced pressure-still tar of 17.3 °A. P. I. gravity and viscosity, S. U. V., of 155 seconds at 100° F., were mixed with 28.7 volumes of uncracked gasoline. This mixture was contacted with dry hydrogen chloride for one hour at 175° F. under 100 pounds pressure. The oil was then stirred at room temperature with 10 per cent by weight of anhydrous aluminum chloride for 4 hours at atmospheric pressure while maintaining the presence of an excess of dry hydrogen chloride. The sludge was permitted to settle and the sour oil was then treated as in the first example. The yield of finished oil was found to be 80.7 volumes. This oil had the following tests:

|                                  | Product |
|----------------------------------|---------|
| 50 Gravity: °A. P. I.            | 20.7    |
| Viscosity, S. U. V.: 100° F      | 290     |
| 210                              | 49      |
| Viscosity index (Dean and Davis) | 65      |
| 55 Flash, O. C.: °F              | 310     |
| Fire, O. C.: °F                  | 370     |
| Pour: °F                         | -5      |
| Color, N. P. A.                  | 6.0     |
| Carbon residue: Per cent         | 0.72    |

60 This example shows a good yield of lubricating oil of fair quality from a tar.

*5. Treatment of reduced pressure-still tar*

One hundred volumes of reduced pressure-still tar of 16.4 °A. P. I. gravity and viscosity, S. U. V., of 160 seconds at 100° F., were mixed with an equal volume of cracked gasoline of 77.4 °A. P. I. gravity. This mixture was contacted with dry hydrogen chloride for 4 hours at ordinary temperature and pressure. The oil was then stirred at 40° F. with 10 per cent by weight of anhydrous aluminum chloride for ten hours at atmospheric pressure. The sludge was permitted to settle and the sour oil was treated as in the first example.

The yield of finished oil was found to be 96.8 volumes, having tests as follows:

|                                  | Product | 5  |
|----------------------------------|---------|----|
| Gravity: °A. P. I.               | 22.0    |    |
| Viscosity, S. U. V.: 100° F      | 216     |    |
| 210                              | 45      |    |
| Viscosity index (Dean and Davis) | 52      |    |
| Flash, O. C.: °F                 | 290     | 10 |
| Fire, O. C.: °F                  | 315     |    |
| Pour: °F                         | +25     |    |
| Color, N. P. A.                  | 8.0     |    |
| Carbon residue: Per cent         | 1.08    |    |

This example shows the improved yields obtainable by the use of cracked instead of uncracked gasoline.

*6. Treatment of light gas oil to yield kerosene*

One hundred volumes of light cracked gas oil 20 from Venezuela crude petroleum were mixed with 20 volumes of amylene and stirred at room temperature with 10 per cent by weight of anhydrous aluminum chloride for 8 hours at atmospheric pressure. An atmosphere of dry hydrogen chloride was maintained over the mixture during stirring. The sludge was permitted to settle and the sour oil was then distilled with 0.1 per cent by weight of hydrated lime. The yield of finished kerosene was found to be 75 volumes having the 30 following comparative tests:

|                                               | Charging stock | Kerosene | 35 |
|-----------------------------------------------|----------------|----------|----|
| Gravity: °A. P. I.                            | 36.5           | 46.0     |    |
| Color, Saybolt                                |                | +25      |    |
| Viscosity, Saybolt thermo-viscosimeter: 60° F |                | 400      |    |
| Flash, T. C. C.: °F                           |                | 139      |    |
| Sulfur (L): Per cent                          | 0.36           | 0.003    | 40 |
| Acid heat: °F                                 |                | 1        |    |
| Distillation, assay:                          |                |          |    |
| Over point: °F                                | 374            | 352      |    |
| End point: °F                                 | 588            | 550      |    |
| Percent at 392° F                             | 10             | 11       |    |
| 500                                           | 88             | 92       |    |
| 590                                           | 97             |          |    |
| 50 percent at: °F                             | 428            | 435      | 45 |

This example shows an increased yield of high grade kerosene by mutual reaction with amylene during refining.

The above examples illustrate a few of the 50 ways in which our invention may be used to improve technical petroleum products. The operating conditions under which the process is carried out can be widely varied without departing from the spirit of our invention. In many cases the 55 procedure may be varied to suit the particular material which is being treated or the particular product which it is desired to produce. Some of these variations have been outlined in the preceding discussion. Others will be immediately 60 evident to those skilled in the art.

Reference is made to our copending application, Serial No. 628,446, filed March 18, 1933, which discloses treatment of oil stocks with a halogenated hydrocarbon in the presence of aluminum chloride.

What we claim is:

1. The process of obtaining an improved lubricating oil in high yield which comprises treating a mixture of a relatively high boiling petroleum stock and a lower boiling petroleum stock at a temperature not above about 300° F. with aluminum chloride in the presence of added HCl to produce a synthetic lubricating oil stock of characteristics intermediate those of the two 75

- original stocks and in yield substantially greater than is obtainable by a similar separate treatment of the two original stocks, settling out the bulk of aluminum chlorid sludge formed, decanting, decomposing the traces of aluminum chlorid sludge that remain in suspension in the decanted liquid by agitating the oil with dilute sulfuric acid, separating the acid, contacting with clay and filtering.
- 10 2. The process of claim 1 wherein sulfuric acid of .5 to 20 per cent strength is employed.
3. The process of obtaining an improved lubricating oil free from impurities and in high yield which comprises mixing a relatively high 15 molecular weight petroleum stock with a lower molecular weight petroleum stock, treating the mixture with aluminum chlorid in the presence of added HCl at a temperature not above about 300° F. to produce a synthetic lubricating oil
- 20 stock of characteristics intermediate those of the two original stocks and in yield substantially greater than that obtainable by a similar separate treatment of the two original stocks, settling out the bulk of aluminum chlorid sludge remaining 25 in the stock, decanting, decomposing traces of aluminum chlorid sludge remaining in the decanted liquid by heating with a small amount of clay to a temperature in the general neighborhood of 450° F. in the presence of a small 30 amount of clay and about 0.6 pounds of lime per acid number per barrel and removing the products of decomposition by filtering to secure
- a refined lubricating oil of the character described.
4. In the production of improved lubricating oils by treatment of admixed unrefined stocks of different hydrocarbons in the presence of aluminum chlorid to give a synthetic product containing suspended aluminum chlorid sludge, the process of finishing which comprises settling the product of the aluminum chlorid treatment to remove the bulk of the aluminum chlorid sludge 10 therein, decanting, decomposing the remaining aluminum chlorid sludge with dilute sulfuric acid, separating the acid, contacting with clay and filtering.
5. The process of claim 4 wherein the acid 15 strength is about 5 to 20 per cent.
6. In the process of obtaining a refined pure lubricating oil from mixtures of unrefined stocks with the aid of aluminum chlorid the finishing procedure which comprises settling out from the 20 aluminum chlorid treatment product the bulk of aluminum chlorid sludge, decanting, decomposing traces of aluminum chlorid sludge remaining in suspension in the decanted liquid by heating to a temperature in the general neighborhood of 25 450° F. with a small amount of clay and with about 0.6 pounds of lime per acid number per barrel and filtering to remove products of decomposition, to secure a pure oil of the character described.
- 30

EUGENE AYRES.  
HERSCHEL G. SMITH.

CERTIFICATE OF CORRECTION.

Patent No. 2,019,037.

October 29, 1935.

EUGENE AYRES, ET AL.

It is hereby certified that error appears in the printed specification of the above numbered patent requiring correction as follows: In the drawings, Sheet 2, Fig. 2, as shown below should appear as a part of the Letters Patent:

Oct. 29, 1935.

E. AYRES ET AL

2,019,037

MANUFACTURE OF IMPROVED HYDROCARBON PRODUCTS

Filed March 10, 1932

2 Sheets-Sheet 2



Fig. 2

Inventors

Eugene Ayres  
Herschel G. Smith

By *G. M. Haughton*  
Their Attorney

and that the said Letters Patent should be read with these corrections therein that the same may conform to the record of the case in the Patent Office.

Signed and sealed this 26th day of November, A. D. 1935.

Leslie Frazer